

## UNITED STATES PATENT OFFICE.

MANUEL LEVIN, OF BOSTON, MASSACHUSETTS.

## METAL POLISH.

No Drawing.

Application filed May 8, 1923. Serial No. 637,590.

*To all whom it may concern:*

Be it known that I, MANUEL LEVIN, a citizen of the United States of America, and resident of Boston, in the county of 5 Suffolk and State of Massachusetts, have invented new and useful Improvements in Metal Polishes, of which the following is a specification.

This invention relates to polishes and 10 more particularly to polishes, either liquid or paste, for finely finished metals or other smooth and lustrous surfaces.

Metal polishes of usual type depend for 15 their cleaning and brightening action upon an abrasive ingredient which removes the metallic oxides or accumulated dirt and dust by friction, or upon the employment, either with or without an abrasive, of coating materials which are deposited in a thin layer 20 upon the surface to be polished and which of themselves impart the desired gloss.

Much labor is required in using polishes 25 of the first type, particularly when the metal to be polished is heavily oxidized or corroded, while the second form of polish is often objectionable as it obscures or dims the metal itself and is frequently of such a character as readily to be scratched or marred, or rapidly to gather dust, thus necessitating very frequent repetitions of the 30 polishing process.

Principal objects of the present invention are to provide a polish for metals or other highly finished surfaces which removes the 35 metallic oxides or other accumulation from the surface by a true chemical reaction therewith, assisted, if desired, by the action of a fine abrasive, but without danger of attacking the surface itself even if left in 40 contact therewith for an indefinite period; to provide a polish which will leave the surface clean and without an appreciable coating after the operation is completed; to provide a polish whose ingredients will 45 remain properly mixed and without substantial separation for long periods, and which may again be mixed by slight agitation if separated by an excessive period of standing; and to provide a polish of the 50 class described which contains no inflammable ingredients and which does not emit disagreeable fumes.

Stated briefly, a polish having the above 55 characteristics may be compounded by suspending a suitable pulverulent abrasive in a non-inflammable fluid forming an am-

monium soap in the mixture, and precipitating an insoluble salt of a fatty acid, herein-after termed for convenience an insoluble soap, upon or around the suspended particles or abrasive, the insoluble soap having a specific gravity slightly less than that of the fluid vehicle employed so that it tends to float the suspended abrasive. In place of insoluble soap or in addition thereto, an insoluble salt, such for example as aluminum silicate which will thicken the mixture or form a jell, may be precipitated in the water with its suspended particles of abrasive. The aluminum silicate may be precipitated 60 by adding any suitable aluminum salt to a solution of sodium silicate in the mixture, and acts in place of or as an auxiliary to the soluble soap to prevent settling or separation of the abrasive from the liquid vehicle 65 in which it is suspended.

The ammonium soap, or soaps, has a triple function in the compound. First, it acts to thicken it to some extent, thus supplementing the supporting action of insoluble soap, or jellied salt; second, it breaks down by evaporation of ammonia when exposed in a thin film in the air, thus freeing the fatty or other acids from which it is 70 formed, and third, when employed for polishing non-metals, in the manner of an ordinary soap. When the polish is used for brightening metal, these acids recombine 75 with any metallic oxides or other compounds upon the surface of the metal, the resulting 80 metallic soaps being readily removable by rubbing so as to leave the surface bright and clean. When applied to non-metallic surfaces the ammonium soap has more or less the function of an ordinary detergent 85 for removing dirt from such surfaces, the breaking down of the soap and the liberation of the fatty acids furnishing an agency well adapted to soften or dissolve accumulation of dirt upon the surface to be polished. 90

The acids which are liberated from the ammonium soap are not strong enough to attack clean or non-corroded metallic or other polished surfaces so that when the surfaces have once been cleaned the chemical reaction ceases. 95

The abrasive in the compound functions in the ordinary manner but is particularly effective when combined with the ammonium soap as it then acts mechanically to remove the insoluble soaps of the metallic ox- 100

60

65

70

75

80

85

90

95

100

105

110

ides as they are formed and constantly exposes fresh surfaces to the action of the acid liberated.

The abrasive which I prefer to use for making a polish for metal or similar surfaces is finely pulverized silex or commercial silicon dioxide ( $SiO_2$ ), although other and generally equivalent materials, as for example flour emery, carborundum, or the like, may be employed if desired. When intended primarily for polishing non-metallic surfaces, powdered pumice, rotten-stone, rouge or other relatively soft abrasive may be substituted for the silex.

I find that water forms a very satisfactory fluid vehicle for the other ingredients particularly when mixed with an alcohol in varying percentages, such fluid vehicle being abundant, substantially neutral in action, and non-inflammable. I contemplate however, that other liquid vehicles having generally similar characteristics may be used, but I regard it as important that the vehicle selected be substantially non-inflammable, although liquids, such as pure alcohol, not subject to the rapid emission of inflammable or explosive fumes, may at times be employed to advantage.

Preferably I employ from five to thirty per cent of alcohol (either methyl or ethyl) with the water for the reason that the alcohol increases the rate of evaporation of the water and ammonia from the film of polish when applied to a surface, thus facilitating the liberation of the fatty acids and increasing the rate at which the metallic oxides or other accumulations upon the surface are attacked.

The soaps, both soluble and insoluble, are preferably formed in the mixture by the action of suitable reagents upon a fatty acid or acids forming an ingredient thereof. The term "fatty acid" as herein employed is not used in its more restricted chemical sense as including only homologues of formic acid, of which stearic acid is a well known example, but as embracing any other of the acid derivatives of the fats or fatty oils, such for example as oleic acid, commercially known as red oil.

I prefer to use those fatty acids having a relatively low melting point, as their compounds with the metals, as well as any unused surplus, may more easily be removed from the metallic surfaces than when the fatty acids of higher melting point are employed. However, various mixtures of the high and low melting point fatty acids are found to give excellent results.

For precipitating the insoluble soap, I prefer to use lime as the reagent, although other salts of calcium, as well as salts of iron, copper, etc., or mixtures thereof may be employed and give satisfactory results.

The polish may readily be perfumed by

adding any desired essential or aromatic oil to the alcohol before mixing it with the water.

In compounding the polish I find it convenient to take about twenty-five gallons of water and add thereto about nine gallons of commercial oleic acid. With these liquids I mix about five hundred pounds of finely pulverized silex, pumice or other selective abrasive, adding the abrasive slowly and with constant stirring. I then add about two and one-half gallons of common aqua ammonia (26 degree Baumé) while continuing to stir the mixture. A stronger or weaker ammonia may be used, but in such case the amount employed should be varied accordingly to ensure an excess to free ammonia sufficient to combine with all the fatty acid. When the compound has attained an even, pasty consistency I add about twenty-nine gallons of lime water, continuing to stir the mixture for about fifteen minutes until the lime water has been incorporated. The lime water should be added slowly while thoroughly agitating the mixture in order to secure even precipitation of the lime soap.

In place of lime water, calcium chloride or other water soluble calcium salt may be used, or in fact any other metallic oxide or hydroxide or other salt which will form an insoluble soap with the fatty acid.

I have contemplated the addition of caustic soda or potash as seemingly desirable ingredients of the polish for the reason that these reagents tend to prevent separation of the solid and liquid components of the compound for an indefinite period, but believe that the advantages thus obtainable are more than offset by the tendency of the soda or potash soaps to remain upon the surface after the polishing operation has been completed, thus dulling the shine or gloss. I therefore prefer to omit such reagents from my polish, although it is possible that they might be found desirable under some circumstances.

The polish prepared as above described is placed in suitable bottles, jars or other containers for sale and use, and although it may be found upon prolonged standing that the heavier particles tend to some extent to separate from the liquid, a slight shaking or stirring is sufficient to restore it to its original condition.

The polish is conveniently applied by placing a small quantity, diluted with water if desired, upon a cloth or pad and applying it to the surface to be cleaned with gentle rubbing or friction. Far less labor is required to obtain the desired luster or gloss than with polishes depending entirely upon the action of an abrasive for their effect, while finely polished surfaces are less likely to be scratched or injured.

After the dirt or oxides have been re-

moved from the surface, the latter is wiped with a soft cloth to remove surplus polish and the products arising from the employment of the polish, thus leaving the surface 5 with a clean and brilliant luster. When the surface is comparatively smooth and free from pits, rubbing may be dispensed with entirely, as the surface film is quickly removed by the chemical and physical action 10 of the fatty acids alone.

While a polish comprising the above noted ingredients in substantially the proportions indicated appears to give the best results, I contemplate changes both in the 15 specific ingredients employed and in the proportions in which they are used as within the scope of my invention.

I claim:

1. A polish comprising finely divided abrasive material having its particles surrounded with the ammonium and calcium soaps of oleic acid. 20

2. A polish comprising water, alcohol, finely divided abrasive material, an insoluble soap, and an ammonium soap. 25

3. A polish comprising a fluid vehicle consisting of water and alcohol, and a finely divided abrasive suspended therein, the particles of the abrasive being surrounded with calcium and ammonium soaps of a fatty 30 acid.

Signed by me at Boston, Massachusetts, this 3rd day of May, 1923.

MANUEL LEVIN.